

F. W. HOCHSTETTER.

PROCESS AND APPARATUS FOR MAKING A TRANSLUCENT MEDIUM FOR USE IN THE

PHOTOGRAPHIC ARTS.

APPLICATION FILED NOV. 13, 1919.

1,345,184.

Patented June 29, 1920.



Inventor

Frederick W. Hochstetter,  
Paulsen & Sonnen,

Attorneys

# UNITED STATES PATENT OFFICE.

FREDERICK W. HOCHSTETTER, OF DAYTON, OHIO, ASSIGNOR OF ONE-HALF TO W. L. OHMER, OF DAYTON, OHIO.

## PROCESS AND APPARATUS FOR MAKING A TRANSLUCENT MEDIUM FOR USE IN THE PHOTOGRAPHIC ARTS.

1,345,184.

specification of Letters Patent. Patented June 29, 1920.

Application filed November 13, 1919. Serial No. 337,825.

To all whom it may concern:

Be it known that I, FREDERICK W. HOCHSTETTER, a citizen of the United States, residing at Dayton, in the county of Montgomery and State of Ohio, have invented certain new and useful Improvements in Processes and Apparatus for Making a Translucent Medium for Use in the Photographic Arts, of which the following is a specification, reference being had therein to the accompanying drawing.

The principal object of my invention is to provide process and apparatus for making a translucent medium for use in the photographic arts in the place of nitro cellulose compounds now generally used. By nitro cellulose compounds I refer to the various translucent and transparent substances used in photographic and similar arts, many forms of which are termed films.

It is the further object of my invention to provide a medium of translucent character which can not only be used for negatives but also for transparencies and diapositives. The range of usefulness of my invention is only limited so far as the photographic art is concerned, by the limits of the art itself. It is applicable to film purposes for both still photography and moving pictures.

It is one of the objects of my invention, that the translucent medium becomes an integral portion of the photographic negative or other use to which it may be put, as distinguished from the attempts in the past to use translucent supports which were merely temporary and had to be removed from the remainder of the negative before the operation could be complete. My object is to provide a permanent base of translucent character like the ordinary film, which shall be partially fireproof and non-combustible. This is a very material advantage over the present film with its highly inflammable and explosive character incurring great danger in handling, shipping and use, as well as in the course of manufacture.

It is my object to provide a translucent medium which shows no grain whatsoever and is free from any opacity which might detract from the usefulness and beauty of

the resulting images, projections or positives.

Furthermore, I have succeeded in thus making such an advance in the art that the result is not only translucent, without grain and non-combustible, but also I have been able to use the ordinary material found on the market, such as paper of varying characters, of varying methods of manufacture, of varying lengths of fiber or lengths of material which have composed the paper and make up its structure. In accomplishing these several objects, I have not affected the rapidity with which positives may be made from the negatives, nor affected the question of projection of images from film in moving pictures where the film is made up of my translucent material.

A further object of my invention is to so provide such translucent medium that no unpleasant refraction would be encountered in the case of projection of moving pictures due to any refractive properties which might either be left in my translucent medium or created by my process of producing it.

I first subject the paper, or other medium which I may employ as a base for treatment, to a combination of absolute alcohol, 4 oz., and castor oil, 1 oz., maintained at 110° F. I apply this compound to the paper at the rate of approximately 1 ft. per second. I prefer this rapid rate to secure the best result. The paper thus treated is passed over heated rolls and then conveyed into a chamber where the temperature is at 100° F., where it is passed into a solution of vaseline and mineral naphtha maintained at a temperature of 100° F. I then pass the paper over cold rollers and then between soft buffers, in a third chamber maintained at normal temperature.

As an example of the machine that I employ for this process, reference is made to the figure of the accompanying drawing.

In this figure, 1 designates a pipe which conveys the combined solution, at 110° F., of alcohol and castor oil, to a tank 2. The amount of the compound admitted to tank 3 is determined by the pet cock 4. The

compound is maintained at the level 5 in the tank 3, in which the rollers 6 and 7 turn, conveying a thin film of the liquid against the paper strip 8 passing between the rolls 6 and 7 and the roll 9. This paper strip is unrolled from the supply roll 10 around a guide roll 11. After being treated with the first compound, it passes over the heated rollers 12, 12, through the guide rolls 13, 13, 10 out of compartment A, which is maintained at 110° F. temperature, into compartment B, which is maintained at 100° F. temperature. Upon passing into compartment B, the paper is conveyed over roll 14, under roll 15, through a bath 16 in the tank 17. This bath is composed of vaseline and mineral naphtha at 100° F. temperature, as explained above. The paper is conveyed over the roll 18, out of the bath 16, into compartment C, passing between the cold rollers 19 and 20 and between the buffers 21 and 21, which reduce it to normal temperature and give it a smooth finish respectively. Whence the paper strip 8 passes to the roll 23, after 25 which it may be sensitized or treated as may be desired for photographic purposes.

In the foregoing compounds and process, and the elements of the machine for executing the process, I do not desire to be confined to the specific materials and methods and elements related, but simply state these factors as illustrative of a preferred and successful form of my invention. I do not intend to thereby limit myself, but consider 30 within the purview of my invention all the equivalents of such factors.

For instance, while I have mentioned paper, I do not intend to confine myself to that medium alone, because my process is 40 applicable to other mediums of opaque character which it may be desired to make translucent.

Having thus fully described my invention, what I claim as new and desire to secure by 45 Letters Patent, is:

1. In combination, a tank, means for conveying a strip of material therethrough, a plurality of heated rollers, a second tank, means adjacent thereto for conveying a 50 strip of material therein, cold rollers and buffers, whereby said combination effects a change in the character of said material.

2. In combination, means for supporting a roll of material, a tank, coöoperating means 55 with the said tank for conveying said material thereto, a plurality of heated rollers, a second tank, means for conveying material thereto, cold rollers, buffers and means for supporting a roll of the finished 60 material, whereby said combination effects a change in the character of said material.

3. In combination, means of supporting a roll of material, a tank, means of supplying said tank with a compound, means of conveying said material into said tank and out 65

again, a plurality of heated rollers, guide rolls, a second tank, means of conveying said material in and out of said tank, cold rollers between which said material passes, buffers between which said material passes and a winding reel, whereby said combination effects a change in the character of said material. 70

4. In a process of making paper translucent, passing said paper into a compound for that purpose, moving said paper over heated rollers, passing said paper between guide rolls, all in a temperature of 110° F., passing said paper into a finishing solution in a chamber the temperature of 100° F., 80 passing said paper into a chamber of normal temperature, moving said paper between cold rollers, rolling said paper and buffing said paper. 75

5. In a process of making paper translucent, passing said paper into a temperature above normal of the surrounding air, treating said paper to make it translucent, passing it over hot rollers, passing it into a chamber of lower temperature but still 90 above normal, giving it a finishing treatment to make it translucent, passing it into a chamber of normal temperature, treating it with cold rollers and buffing it. 85

6. In a process of making paper translucent, passing said paper into a temperature above normal of the surrounding air, treating said paper to make it translucent, passing it over hot rollers, passing it into a chamber of lower temperature but still 100 above normal, giving it a finishing treatment to make it translucent, passing it into a chamber of normal temperature, treating it with cold rollers, buffing it and winding it on a reel. 95

7. In a process of making paper translucent, passing it into a chamber of approximately 110° F., treating it with a combination of absolute alcohol and castor oil, passing it over heated rollers, passing it into a 110 temperature of approximately 100° F., treating it with a compound of vaseline and mineral naphtha at approximately a temperature of 100° F., passing it into a chamber of normal temperature, rolling it with 115 cold rollers and buffing it. 105

8. In a process of making paper translucent, passing it into a chamber of approximately 110° F., treating it with a combination of absolute alcohol and castor oil at the 120 rate of approximately 1 ft. per second, passing it over heated rollers, passing it into a temperature of approximately 100° F., treating it with a compound of vaseline and mineral naphtha at approximately a temperature of 100° F., passing it into a chamber of normal temperature, rolling it with 125 cold rollers and buffing it. 115

9. In a process of making paper translucent, passing it into a chamber of approxi- 130

mately 110° F., treating it with a combination of 4 oz. of absolute alcohol and 1 oz. of castor oil at the rate of approximately 1 ft. per second, passing it over heated rollers, 5 passing it into a temperature of approximately 100° F., treating it with a compound of vaseline and mineral naphtha at approxi-

mately a temperature of 100° F., passing it into a chamber of normal temperature, rolling it with cold rollers and buffing it. 10

In testimony whereof, I affix my signature.

FREDERICK W. HOCHSTETTER.